

Nov. 11, 1924.

1,515,276

G. R. RICH

TAPPET

Filed April 8, 1924

Fig. 1.



Fig. 2.



Fig. 3.



Fig. 4.



Fig. 5.



Inventor:  
George R. Rich,  
by Charles O. Harvey  
his Atty.

## UNITED STATES PATENT OFFICE.

GEORGE R. RICH, OF BATTLE CREEK, MICHIGAN, ASSIGNOR TO RICH STEEL PRODUCTS COMPANY, OF BATTLE CREEK, MICHIGAN, A CORPORATION OF CALIFORNIA.

## TAPPET.

Application filed April 8, 1924. Serial No. 704,949.

To all whom it may concern:

Be it known that I, GEORGE R. RICH, a citizen of the United States, and a resident of Battle Creek, Calhoun County, and State 5 of Michigan, have invented certain new and useful Improvements in Tappets, of which the following is declared to be a full, clear, and exact description.

This invention relates to valve tappets 10 for internal combustion engines and its principal object is to protect the bearing face of the head of the tappet and provide against rapid deterioration thereof by the action of the cam thereon, particularly when the tappet 15 seat is new or when the motor or engine is first operated.

It is well known that because of improper lubrication, improper alignment of the cam shaft and of the tappets, and because of imperfections in the bearing faces of the cams 20 and for various other reasons, the cams rapidly wear away the true bearing faces of the tappet heads, thereby interfering with the proper lifting and seating of the valves, 25 and causing annoying clicking noises between the tappets and valves and between the tappets and cams.

In the usual process of machining and 30 hardening valve tappets the hard outer surface portion is often removed in grinding the bearing face of a tappet head thereby exposing the relatively softer metal of the head to the action of the cam, with the result that the cam soon wears away the true 35 bearing face of the tappet. In the operation of a motor at normal speed the cam travels over the head of the tappet so rapidly and in such rapid succession that the lubricating oil scarcely has time to cover 40 the bearing face of the tappet head between the successive revolutions of the cam, the result being undue wear and permanent injury to the true bearing face of the tappet head. Moreover when newly installed, 45 the associated bearing surfaces of the tappets and cams, although nicely ground, are raw, and under the microscope present innumerable pits and sharp edges; these raw faces must be worn down to obtain smoothness of action, and the wear occasioned 50 makes a difference in the lifting and seating movements of the tappet.

I have discovered that greater efficiency 55 of operation is obtained, greater precision and smoothness of action results and that

noise is minimized, by providing a protective metallic covering or surfacing for the bearing face of the tappet head, which covering fills the pores at the surface and presents a smooth anti-friction surface to 60 the cam, which surface, under the influence of the cam, is rendered still smoother, the anti-friction material is permanently embedded in the pores and the whole surface becomes burnished, thereby providing a permanent smooth bearing surface, on which the friction between the cam and tappet is 65 reduced to a minimum.

In the course of my experiments I have found that by tinning the bearing face of 70 the tappet head, excellent results are obtained and further, that by the use of composite anti-friction bearing materials, such as tin and pulverized bronze, a most effective result is obtained. In some cases 75 the use of pulverized iron, united to the bearing face by a more fusible metal, such as tin, has served the purpose with a remarkable degree of success.

To such ends this invention consists in 80 a valve tappet for internal combustion engines having a head formed with a bearing surface, to which is applied an anti-friction bearing material that covers the raw metal and protects it against the abrasive action of the cam. It further consists in 85 a valve tappet having a head formed with a bearing surface and a coating thereon united with said bearing surface and forming a protective cover therefor. It further 90 consists in a valve tappet formed with a head having a tinned bearing surface. It further 95 consists in a valve tappet formed with a head having a bearing surface covered with pulverized bronze united thereto by a readily fusible metal. It further consists in the several other novel features hereinafter fully set forth and claimed.

The invention is clearly illustrated in the drawing accompanying this specification, in 100 which:

Fig. 1 is a side elevation of a tappet, embodying a simple form of the present invention, and an associated cam, the cam shaft being shown in cross-section; Fig. 2 is a side 105 elevation of the parts seen in Fig. 1 looking at right angles thereto; Fig. 3 is an end view of the tappet seen in Fig. 1 with a portion of the coating or surface material removed from the bearing face of its head; 110

Fig. 4 is a detail, fragmental, longitudinal section through the tappet, showing its condition prior to the application of the protective covering thereto, and Fig. 5 is a view similar to Fig. 4 with the addition of the protective covering thereto.

Referring to said drawing, which illustrates one embodiment of the present invention, the reference character 6 designates the 10 valve tappet forming the subject matter of this specification, 7 designates an associated cam, and 8 a fragment of the cam shaft upon which the cam is formed. In accordance with the usual practice the tappet comprises the stem portion 9 which is ordinarily mounted in suitable bushings or bearings in the motor and said stem may be hollow if desired, as seen in Figs. 4 and 5, although this is not essential to the present invention. 15 20 The tappet head 10 is shown as of the mushroom type and is formed with the bearing face 11, with which the cam 7 contacts. The bearing face 11 of the tappet head is shown as flat but this is not necessary as it may be crowned if so desired and in many cases this is preferred. The tappet is held down upon the cam by a spring (not shown) as is well understood and the upper end of the tappet is provided with means for engaging with 25 or for actuating the valve, but as these parts have no bearing upon the present invention they will not be described in detail. As is well understood, the cam shaft rotates, and rotates the cam 7 and during each rotation 30 of the shaft the high part of the cam lifts the tappet, thereby unseating the valve, and the spring lowers the tappet when the high part of the cam passes the head of the tappet. 35 40 As is customary, the tappet is formed from a rod of suitable metal preferably from steel alloy, and the head is formed upon the stem by suitable dies. In the process of hardening, machining and finishing the tappet, the bearing face 11 is ground off nicely, but when observed under a microscope, innumerable pits and sharp edges and rough spots are observed on said bearing face. The same may be said of the cam. When 45 50 the raw bearing face of the cam rubs upon the raw bearing face of the tappet head, especially if they are not properly lubricated, the bearing face of the tappet head is rapidly and unevenly worn away and sometimes edges of the cam cut grooves in the bearing face of the tappet head, with the result that its true bearing face is distorted and worn away to such a degree that the lifting and seating of the valve by the tappet is changed, thereby reducing the efficiency of the motor, besides producing annoying, clicking noises.

In place of permitting the raw bearing surfaces of the cam and tappet head to contact with each other, I coat the bearing face

of the tappet head with a metallic protective material 12, which in one form may comprise tin, and in another form may comprise tin containing pulverized iron, but in its preferred form it comprises tin containing pulverized bronze. Said coating may, however, comprise any anti-friction material that may be united with the bearing face of the tappet head and as an example, Babbitt metal may be employed.

In the process of forming a tappet containing the present invention, the tappet is first formed, ground and finished in the ordinary manner, after which the coating is applied to its head. In applying the coating, the coating material is kept upon a hot plate, and the tappets are heated up to a temperature of approximately 200 degrees; the bearing face of each tappet is then dipped into a proper solution of acid and 20 immediately placed on the hot plate containing the surfacing material, which plate is preferably kept at a temperature of approximately 450 degrees, and the bearing face of the tappet is rubbed over and 25 through the surfacing material contained on the plate until the quantity required, unites with the bearing face of the tappet, after which the face is immediately wiped off with a piece of felt or like material and the 30 tappet is dropped into a cooling bath.

When composite metals such as tin and bronze are used for coating the bearing face of the tappet head, the bronze is pulverized and it is added to the tin, as much bronze 35 being used as will be absorbed by the tin. The tin melts at the temperature to which the surfacing material is exposed, but the bronze does not, necessarily, but is transferred in its pulverized state, to the bearing 40 face of the tappet when the latter is rubbed upon the hot plate containing the materials, and the bronze is thereby united to the bearing face by the tin. The use of bronze has been found to be highly desirable because 45 of its anti-friction qualities.

From my observations of the results obtained by the use of a protective covering for the bearing faces of tappet heads, I find that the action of the cam on the bearing 50 face is to impact or force the surfacing material or at least a part of same, further into the pores of the metal and to burnish or polish the bearing face of the tappet head without perceptibly wearing away any of 55 the metal of the head itself. Moreover I have observed that some of the surfacing material is absorbed by the cam, which indicates that both bearing surfaces of the tappet and cam become perfectly smooth 60 without any appreciable wear thereon and without any distortion.

I claim as new, and desire to secure by Letters Patent:

1. A tappet having a head formed with a

ground bearing face adapted for engagement with a cam, said bearing face having a metallic, anti-friction surface protecting material thereon and united therewith.

5 2. A tappet having a head formed with a bearing face, adapted for engagement with a cam, said bearing face being coated with a metallic composition containing pulverized bronze.

10 3. A tappet having a head formed with a

bearing face, adapted for engagement with a cam, said bearing face having pulverized bronze united to it by a more fusible metal.

4. A tappet having a head formed with a ground bearing face, adapted for engagement with a cam, said bearing face having pulverized anti-friction metal united to it by a more fusible metal. 15

GEORGE R. RICH.